

May 12, 1942.

W. F. WRIGHT

2,283,152

METHOD OF CASTING METAL AND CAST ARTICLE

Filed July 31, 1940



Fig. 1



Fig. 2



INVENTOR

BY *Walter F. Wright*  
*Wood & Wood* ATTORNEYS

## UNITED STATES PATENT OFFICE

2,283,152

## METHOD OF CASTING METAL AND CAST ARTICLE

Walter F. Wright, Wyoming, Ohio

Application July 31, 1940, Serial No. 348,753

4 Claims. (Cl. 22—65)

This invention relates generally to the art of casting metal and is particularly directed to an improved method of casting steel gear and wheel blanks and articles of that general nature.

Many castings are faulty and unusable because they contain shrinkage cavities or pipes. Such faults occurring inside of a casting, sometimes are exposed after the rough article has been machined, and the labor which has been spent in the machine operations prior to the discovery of the fault is wasted when it is necessary to discard the casting. Beyond this, shrinkage cavities which are not exposed during the machining operation provide weakened areas in the casting which sometimes do not come to light until breaks occur.

These cavities occur in castings at the points which are last to solidify. This happens because, as the cooling begins along the walls of the metal and proceeds inwardly from these surfaces, metal is drawn from the portions which still remain fluid and thus, metal is drawn from the inner parts toward the outer, so that, finally an empty space or pipe is left in the center. Although it is not constant, as a general rule, the shrinkage amounts to as much as 5 or 6 per cent.

In the past it has been the practice to provide a plurality of risers or feed heads in such places that any decrease in volume was taken care of by molten metal drawn from one of the plurality of feed heads, the theory being that the final shrinkage cavities or pipes would be in the risers. A casting on the order of a gear blank usually required a number of risers positioned around the rim and another riser positioned near the center of the hub of the casting. If enough risers were used, it was found that the majority of the shrinkage cavities could be corrected by this method. But the correct placing and relative sizes of the different feed heads for one casting often required much study and time, and in some instances, it was found impossible to place the feed heads where they were most needed. Then, too, unless the risers were placed with extreme care with regard to their relative proportions, it was found that varying degrees of denseness prevailed in the casting.

It has been an object of the present inventor to provide a method of casting which provides a casting having a uniform and maximum density and one which is free from the shrinkage cavities described above, which method does not require the use of the riser or feeder system on the rim above referred to.

In the fulfillment of this objective, it has been discovered that the casting mass should be arranged so that it increases from the outermost portions to the innermost. Accordingly as solidification takes place; that is, as the casting

cools, the cooling occurs from the outer portion toward the inner portion; that is, retrogressively. As the metal in the outer portion cools or shrinks, it draws from the inner portion proceeding in this manner to a central riser from which the central portion of the casting or the most massive portion draws metal in the final cooling phase. Obviously, the less massive the casting portion is, the faster it will cool.

10 In this procedure, the mold is rotated and centrifugal force constantly presses the molten metal outwardly into the rim or margin of the casting. This, plus the inwardly progressing cooling action, produces a metal casting which is solid throughout from the extremities to the central mass with a single central riser sufficing to supplement the metal last to shrink.

It is another object of this inventor to provide a casting having its mass arranged as set forth; 20 that is, with the outer extremities of less mass than the inner. The mass of the casting increases uniformly from the outer portion to the inner.

Other objects and advantages of my invention 25 will be more fully set forth in a description of the drawing, forming a part of this specification, in which:

Figure 1 is a sectional view taken through a mold and casting embodying my invention.

30 Figure 2 is a plan view of the rough finished casting.

Figure 3 is a fragmentary sectional view taken on line 3—3 of Figure 2.

Figure 4 is a fragmentary sectional view taken 35 on line 4—4 of Figure 2.

Figure 5 is a fragmentary sectional view taken on line 5—5 of Figure 2.

Figure 6 is a fragmentary sectional view taken 40 on line 6—6 of Figure 2.

The casting shown in the drawing is a gear blank. For this kind of casting it is especially desirable to have an article which is of maximum uniform density and free of pipes. As disclosed in Figure 1, the mold, indicated at 1, is mounted on a rotating table 2. The table is revolved by means of a bevel gear 3, pinned to a central shaft 4 and driven by means of a bevel gear 5. The table may be supported on a bearing as at 6.

The mold, constructed according to the usual 50 foundry practice, comprises a circular flask formed in two pieces which are connected at a horizontal joint. The upper piece, referred to as the cope flask, is indicated at 7, and the lower piece, referred to as the drag flask, is indicated at 8. The respective flasks have sand molds formed therein, indicated generally at 9. In this instance a core 10 is provided for the central opening in the gear blank.

As shown in Figure 1, the sand in the cope 55 flask is formed to provide a riser chamber 11.

This view may be treated as showing the casting immediately after formation and prior to removal from the mold. The casting comprises a hub portion 12, spokes 13 and a rim 14. The dot-dash line 15, dividing the riser from the hub of the gear blank, defines the line through which a cut is made to separate the riser from the hub after the article is removed from the mold.

Regarding the article, it may be seen that in cross section the riser 11 comprises a greater mass than the hub 12, the hub comprises a greater mass than the larger ends of the tapered spokes 13 and the smaller ends of the tapered spokes comprise a greater mass than the rim 14. The mass as measured by cross sectional area, is increased approaching the center. Figures 3 to 6, inclusive, illustrate this point.

In practice, with the mold prepared, the molten metal is poured. The lower section of the hub fills first, then the spokes and rim, and then the upper section of the hub. The pouring continues until the riser is filled and leveled off. Immediately after pouring, the mold is rotated rapidly. Under centrifugal force, the molten metal is thrown outwardly, radially toward the rim. As the molten metal cools, the rim is first to completely solidify, since it has the smallest cross section of the casting. Solidification continues moving inwardly from the smaller sections toward the center of the casting. While the solidification moves inwardly, the outward pressure of the molten metal is kept constant, so that as shrinkage upon solidification occurs, the outward pressure of molten metal supplies the necessary metal to the parts. In other words, the mold is filled from the center and the molten metal is pressed outwardly, radially, while solidification takes place retrogressively against the feeding pressure.

The above disclosed method of casting may be utilized on other castings (not shown) such as pulley wheels and flanged car wheels. Pulley wheel blanks may be cast in the same manner as the above described gear blank. Flanged car wheel blanks, using the same method, may be cast with the flange on the lower side of the mold so that the flange is filled with molten metal before the rim is completely filled. Here, the flange is designed so that its cross sectional area is less than the rim's area.

It will be apparent to those skilled in the art that many other articles may be cast according to this method. Some articles which do not readily lend themselves to the necessary design, i. e., a design having the mass increasing from the outer edges toward a central point, may be designed with their mass proportioned according to this invention and after they are cast, machined to the wanted proportions. This latter method, although more expensive, is well worth the added cost when it is necessary to turn out a casting which has to be guaranteed against internal cavities. In most instances, the extra machining is confined to the center sections and takes no more time to accomplish than it did to cut off the many risers used in past methods.

Having described my invention, I claim:

1. The method of casting steel to provide an article of the type having a hub, a rim, and a connection portion, comprising; the steps of, providing a mold in which the cross-sectional area

of the mold cavity increases from the rim portion to the hub portion, providing a riser cavity at the center of the mold to feed the central cavity thereof, and rotating the mold to cause the molten steel to be urged outwardly whereby the steel solidifies at the rim portions first and solidification proceeds inwardly to the center portion, which portion being the last to cool is fed from the central riser.

2. The method of casting which comprises the step of preparing, in a sand mold, a cavity having a central chamber, a rim chamber and at least one chamber interconnecting the rim passageway with the central chamber, the cross-sectional areas through the passageways being so dimensioned relative to one another that in the absence of forced cooling and through normal dissipation of heat, as distinguished from artificial cooling or chilling, molten metal introduced into the mold cavity through its central chamber and forced outwardly under centrifugal force to the rim and interconnecting chamber will solidify at a given point in any chamber and thereby close said chamber against further movement of molten metal through it only after the metal has solidified in the portions of the mold cavity which are more remote from the central chamber.

3. A method of casting steel or steel alloys which comprises preparing, a sand mold devoid of chilling members or artificial cooling means, and providing in said mold a molding cavity which is made up of a central chamber, a rim chamber and at least one chamber interconnecting the rim chamber and the central chamber, the said rim chamber, connecting chamber, and central chamber being so dimensioned relative to one another as to cross-sectional areas therethrough that molten steel introduced into said central chamber and delivered centrifugally to said rim chamber and interconnecting chamber will solidify throughout the cross-sectional area at any given point in any of said chambers only after the steel has solidified at points in said chambers more remote from said central chamber whereby the steel in the central chamber is the steel last to cool and prior thereto remains in fluid state to serve as a reservoir supplying molten steel to offset the shrinkage attending the solidification of the steel in the cavities remote from the central chamber, then introducing molten steel into said mold cavity through the central chamber and forcing said molten steel outwardly under centrifugal force whereby the metal solidifies retrogressively while under centrifugal force.

4. A steel casting of the type having a hub, a rim and a connecting portion, said casting formed in a sand mold of a shape providing a casting, the cross-sectional areas of which throughout the various portions increase gradually from the rim to the hub and formed of molten steel introduced into the entire mold cavity centrally thereof and forced outwardly centrifugally whereby the cooling takes place retrogressively from the rim portion to the hub, and the steel in the hub portion is the last to cool and prior thereto remains in fluid state to serve as a reservoir supplying molten steel to offset the shrinkage attending the solidification of the steel in the cavities most remote from the hub portion.

WALTER F. WRIGHT.